# EUROPEAN PATENT APPLICATION

(11) **EP 4 786 615 A1**
(43) Date of publication of application: **05.08.2026**
(21) Application number: 23954189.9
(22) Date of filing: 26.09.2023
(51) Int. Cl.: C22C 29/08

(54) **CEMENTED CARBIDE**

(71) Applicant: Sumitomo Electric Industries, Ltd., Osaka-shi, Osaka 541-0041 (JP)
(72) Inventor: KIDO, Yasuki, Osaka-shi, Osaka 541-0041 (JP); KIMURA, Yoshihiro, Osaka-shi, Osaka 541-0041 (JP); PASEUTH, Anongsack, Osaka-shi, Osaka 541-0041 (JP)
(74) Representative: Boult Wade Tennant LLP
(86) International application number: PCT/JP2023/035009
(87) International publication number: WO 2025/069213

(57) **Abstract**

A cemented carbide includes a plurality of tungsten carbide grains and a binder phase, wherein the cemented carbide includes 89 volume% or more of the tungsten carbide grains and the binder phase in total, the cemented carbide includes 1.8 volume% or more and 20.0 volume% or less of the binder phase, the binder phase includes cobalt, the cemented carbide includes 1.0 mass% or more of the cobalt, and a hardness of the binder phase at 25°C as measured by a nanoindenter method is 7.0 GPa or more.

## Description

### TECHNICAL FIELD

The present disclosure relates to a cemented carbide.

### BACKGROUND ART

Conventionally, a cemented carbide including a plurality of tungsten carbide grains and a binder phase has been used as a material of a cutting tool (PTL 1).

### CITATION LIST

### PATENT LITERATURE

PTL 1: Japanese Patent Laying-Open No. 2004-131769

### SUMMARY OF INVENTION

A cemented carbide according to the present disclosure is a cemented carbide comprising a plurality of tungsten carbide grains and a binder phase, wherein
the cemented carbide includes 89 volume% or more of the tungsten carbide grains and the binder phase in total,
the cemented carbide includes 1.8 volume% or more and 20.0 volume% or less of the binder phase,
the binder phase includes cobalt,
the cemented carbide includes 1.0 mass% or more of the cobalt, and
a hardness of the binder phase at 25°C as measured by a nanoindenter method is 7.0 GPa or more.

### BRIEF DESCRIPTION OF DRAWINGS

[Fig. 1] Fig. 1 is a diagram schematically showing one cross section of a cemented carbide according to one embodiment of the present disclosure.

### DETAILED DESCRIPTION

### [Problem to be Solved by the Present Disclosure]

With increased difficulties in cutting of workpieces in recent years, a cutting tool have been used in a severe condition. Therefore, cemented carbide, which is used as a substrate of a cutting tool, has been also required to have improved various properties. There has been required a cemented carbide allowing for a long life of a tool particularly even when used as a material of a cutting tool for cutting a high-hardness material.

Thus, an object of the present disclosure is to provide a cemented carbide allowing for a long life of a tool particularly even when used as a material of a cutting tool for cutting a high-hardness material.

### [Advantageous Effect of the Present Disclosure]

According to the present disclosure, it is possible to provide a cemented carbide allowing for a long life of a tool particularly even when used as a material of a cutting tool for cutting a high-hardness material.

### [Description of Embodiments]

First, embodiments of the present disclosure will be listed and described.
(1) A cemented carbide according to the present disclosure is a cemented carbide comprising a plurality of tungsten carbide grains and a binder phase, wherein
   the cemented carbide includes 89 volume% or more of the tungsten carbide grains and the binder phase in total,
   the cemented carbide includes 1.8 volume% or more and 20.0 volume% or less of the binder phase,
   the binder phase includes cobalt,
   the cemented carbide includes 1.0 mass% or more of the cobalt, and
   a hardness of the binder phase at 25°C as measured by a nanoindenter method is 7.0 GPa or more.
   According to the present disclosure, it is possible to provide a cemented carbide allowing for a long life of a tool particularly even when used as a material of a cutting tool for cutting a high-hardness material.
(2) In (1), the binder phase may further include a first element, and
   the first element may be at least one element selected from a group consisting of silicon, phosphorus, germanium, tin, rhenium, ruthenium, osmium, iridium, and platinum. Thus, it is possible to provide a cemented carbide allowing for a longer tool life of the cutting tool particularly even in cutting of a high-hardness material.
(3) In (2), in the binder phase, a percentage {M1/(M1+M2)}×100 of a mass M1 of the first element with respect to a total M1+M2 of the mass M1 of the first element and a mass M2 of the cobalt may be 1% or more and 6% or less. Thus, it is possible to provide a cemented carbide allowing for a longer tool life of the cutting tool particularly even in cutting of a high-hardness material.

### [Details of Embodiments of the Present Disclosure]

With reference to figures, the following describes specific examples of a cutting tool according to one embodiment (hereinafter, also referred to as "the present embodiment") of the present disclosure. In the figures of the present disclosure, the same reference characters represent the same or corresponding portions. Further, a dimensional relation such as a length, a width, a thickness, or a depth is appropriately changed for clarity and simplification of the figures, and therefore do not necessarily represent an actual dimensional relation.

In the present disclosure, the expression "A to B" represents a range of lower to upper limits (i.e., A or more and B or less), and when no unit is indicated for A and a unit is indicated only for B, the unit of A is the same as the unit of B.

When a compound or the like is expressed by a chemical formula in the present disclosure and an atomic ratio is not particularly limited, it is assumed that all the conventionally known atomic ratios are included, and the atomic ratio should not be necessarily limited only to one in the stoichiometric range.

### [First Embodiment: Cemented Carbide]

A cemented carbide according to one embodiment of the present disclosure will be described with reference to Fig. 1.

One embodiment of the present disclosure (hereinafter, also referred to as the "present embodiment") is a cemented carbide 3 comprising a plurality of tungsten carbide grains 1 and a binder phase 2, wherein
cemented carbide 3 includes 89 volume% or more of tungsten carbide grains 1 and binder phase 2 in total,
cemented carbide 3 includes 1.8 volume% or more and 20.0 volume% or less of binder phase 2,
binder phase 2 includes cobalt,
cemented carbide 3 includes 1.0 mass% or more of the cobalt, and
a hardness of binder phase 2 at 25°C as measured by a nanoindenter method is 7.0 GPa or more.

According to the present disclosure, it is possible to provide cemented carbide 3 allowing for a long life of a tool particularly even when used as a material of a cutting tool for cutting a high-hardness material. This is presumably due to the following reason.

Cemented carbide 3 according to the present embodiment includes the plurality of tungsten carbide grains 1 (hereinafter, also referred to as "WC grains 1") and binder phase 2, and the total content ratio of WC grains 1 and binder phase 2 in cemented carbide 3 is 89 volume% or more. Thus, cemented carbide 3 has high hardness and strength, and a cutting tool using cemented carbide 3 can have excellent wear resistance and breakage resistance.

Cemented carbide 3 according to the first embodiment includes 1.8 volume% or more and 20.0 volume% or less of binder phase 2, binder phase 2 includes the cobalt, and cemented carbide 3 includes 1.0 mass% or more of the cobalt. Further, the hardness of binder phase 2 at 25°C as measured by the nanoindenter method is 7.0 GPa or more, and binder phase 2 can have excellent hardness under the condition of 25°C (in other words, under a room temperature condition). Thus, the hardness of cemented carbide 3 is improved, with the result that a cutting tool using cemented carbide 3 can have excellent wear resistance particularly even in processing of a high-hardness material.

### << Composition of Cemented Carbide>>

Cemented carbide 3 includes 89 volume% or more of tungsten carbide grains 1 and binder phase 2 in total. Thus, the hardness of cemented carbide 3 can be increased. Cemented carbide 3 may include 90 volume% or more, 91 volume% or more, or 92 volume% or more of tungsten carbide grains 1 and binder phase 2 in total. In cemented carbide 3, the upper limit of the total content ratio of tungsten carbide grains 1 and binder phase 2 may be, for example, 100 volume% or less, 99 volume% or less, or 98 volume% or less. Cemented carbide 3 may include 90 volume% or more and 100 volume% or less, 91 volume% or more and 100 volume% or less, or 92 volume% or more and 100 volume% or less of tungsten carbide grains 1 and binder phase 2 in total.

Cemented carbide 3 includes 1.8 volume% or more and 20.0 volume% or less of binder phase 2. Thus, the hardness and toughness of cemented carbide 3 can be increased. The lower limit of the content ratio of binder phase 2 in cemented carbide 3 may be 2.0 volume% or more, may be 3.0 volume% or more, or may be 4.0 volume% or more. The upper limit of the content ratio of binder phase 2 in cemented carbide 3 may be 19.0 volume% or less, 18.0 volume% or less, or 17.0 volume% or less. Cemented carbide 3 may include 2.0 volume% or more and 19.0 volume% or less of binder phase 2, 3.0 volume% or more and 18.0 volume% or less of binder phase 2, and 4.0 volume% or more and 17.0 volume% or less of binder phase 2.

Cemented carbide 3 according to the first embodiment can consist of the plurality of tungsten carbide grains 1 and binder phase 2. Cemented carbide 3 according to the present embodiment can include another phase (not shown) in addition to tungsten carbide grains 1 and binder phase 2. Examples of the other phase include a carbide, nitride or carbonitride including at least one second element selected from a group consisting of titanium (Ti), tantalum (Ta), niobium (Nb), zirconium (Zr), hafnium (Hf) and molybdenum (Mo). The composition of the other phase is, for example, TiCN, TaC, NbC, ZrC, HfC, or Mo₂C.

Cemented carbide 3 according to the first embodiment can consist of tungsten carbide grains 1, a binder phase 2, and the other phase. Any content ratio of the other phase of cemented carbide 3 is accepted to such an extent that the effects of the present disclosure are not impaired. For example, the content ratio of the other phase of cemented carbide 3 may be more than 0 volume% and 20 volume% or less, may be more than 0 volume% and 18 volume% or less, or may be more than 0 volume% and 16 volume% or less. In this case, the total content ratio of tungsten carbide grains 1 and binder phase 2 in cemented carbide 3 may be 80 volume% or more and less than 100 volume%, may be 82 volume% or more and less than 100 volume%, or may be 84 volume% or more and less than 100 volume%.

Cemented carbide 3 according to the first embodiment can include an impurity. Examples of the impurity include iron (Fe), calcium (Ca), oxygen (O), and sulfur (S). Any content ratio of the impurity in cemented carbide 3 is accepted to such an extent that the effects of the present disclosure are not impaired. For example, the content ratio of the impurity in cemented carbide 3 may be 0 mass% or more and less than 0.1 mass%. The content ratio of the impurity in cemented carbide 3 is measured by ICP emission spectroscopy (Inductively Coupled Plasma Emission Spectroscopy (measurement device: "ICPS-8100" (trademark) provided by Shimadzu Corporation)).

A method of measuring the content ratio [volume%] of tungsten carbide grains 1 in cemented carbide 3 and the content ratio [volume%] of binder phase 2 in cemented carbide 3 is as follows.

(A1) Cemented carbide 3 is cut at any position to expose a cross section. The cross section is mirror-finished using a cross section polisher (provided by JEOL).

(B1) An analysis is performed onto the mirror-finished surface of cemented carbide 3 using a scanning electron microscope-energy dispersive X-ray spectrometry (SEM-EDX) (device: Gemini 450 (trademark) provided by Carl Zeiss) so as to specify elements included in cemented carbide 3.

(C1) The mirror-finished surface of cemented carbide 3 is imaged using the scanning electron microscope (SEM), thereby obtaining a reflected electron image. An imaging region in the captured image is set to the central portion of the cross section of cemented carbide 3, i.e., is set to a position that does not include a portion having a property apparently different from that of a bulk portion such as the vicinity of the surface of cemented carbide 3 (a position with which the imaging region entirely corresponds to the bulk portion of cemented carbide 3). An observation magnification is 5000 times. Measurement conditions are an acceleration voltage of 3 kV, a current value of 2 nA, and a working distance (WD) of 5 mm.

(D1) An analysis is performed onto the imaging region described above in (C1) using the energy dispersive X-ray spectrometer (SEM-EDX) accompanied with the SEM, the distribution of the elements specified as described above in (B 1) is specified in the imaging region, thereby obtaining an element mapping image.

(E1) The reflected electron image obtained as described above in (C1) is loaded into a computer, and is subjected to binarization processing using image analysis software (OpenCV, SciPy). In the image having been through the binarization processing, tungsten carbide grains 1 are shown in white, and binder phase 2 is shown in gray to black. It should be noted that since a threshold value for the binarization is changed depending on a contrast, the threshold value is set for each image.

(F1) The element mapping image obtained as described above in (D1) and the image having been through the binarization processing and obtained as described above in (E1) are superimposed on each other so as to specify respective regions in which tungsten carbide grains 1 and binder phase 2 are present on the image having been through the binarization processing. Specifically, a region, which is shown in white in the image having been through the binarization processing and in which tungsten (W) and carbon (C) are present in the element mapping image, corresponds to the region in which tungsten carbide grains 1 are present. A region, which is shown in gray to black in the image having been through the binarization processing and in which cobalt (Co) is present in the element mapping image, corresponds to the region in which binder phase 2 is present.

(G1) One measurement visual field having a rectangular shape of 24.9 µm × 18.8 µm is set in the image having been through the binarization processing. The above-described image analysis software is used to measure an area percentage of each of tungsten carbide grains 1 and binder phase 2 with the area of the entire measurement visual field as the denominator.

(H1) The measurement described above in (G1) is performed in each of five different measurement visual fields that do not overlap with one another. In the present specification, the average of the area percentages of tungsten carbide grains 1 in the five measurement visual fields corresponds to the content ratio [volume%] of the tungsten carbide grains 1 of cemented carbide 2, and the average of the area percentages of binder phase 2 in the five measurement visual fields corresponds to the content ratio [volume%] of binder phase 2 of cemented carbide 3.

When cemented carbide 3 includes the other phase in addition to tungsten carbide grains 1 and binder phase 2, the content ratio of the other phase of cemented carbide 3 can be obtained by subtracting, from the whole of cemented carbide 3 (100 volume%), the content ratio [volume%] of tungsten carbide grains 1 and the content ratio [volume%] of binder phase 2 measured by the above-described procedure.

As long as the applicant has performed the measurement and the measurement is performed onto the same sample, it has been confirmed that measurement results are small in variation and are not intentional even when the cut portion of the cross section of cemented carbide 3 is freely set, the imaging region described above in (C1) is freely set on the cross section, and the content ratio of tungsten carbide grains 1 and the content ratio of binder phase 2 of cemented carbide 3 are measured a plurality of times in accordance with the above-described procedure.

### <<Binder Phase>>

Binder phase 2 includes the cobalt, and cemented carbide 3 includes 1.0 mass% or more of the cobalt. Thus, excellent toughness can be provided to cemented carbide 3. It should be noted that binder phase 2 may include 50 mass% or more, 60 mass% or more, 70 mass% or more, 80 mass% or more, 90 mass% or more, or 95 mass% or more of the cobalt. Binder phase 2 may consist of the cobalt. Moreover, binder phase 2 may consist of the cobalt and a first element described later. The cobalt in cemented carbide 3 may be present only in binder phase 2. The lower limit of the content ratio of the cobalt in cemented carbide 3 may be 2.0 mass% or more, 3.0 mass% or more, or 4.0 mass% or more. The upper limit of the content ratio of the cobalt in cemented carbide 3 may be 20 mass% or less, 15 mass% or less, 12 mass% or less, or 10 mass% or less. Cemented carbide 3 may include 1.0 mass% or more and 20 mass% or less of the cobalt, 2.0 mass% or more and 15 mass% or less of the cobalt, or 3.0 mass% or more and 12 mass% or less of the cobalt.

A method of measuring the content ratio of the cobalt in cemented carbide 3 is as follows. First, the imaging region is set in the same manner as in (A1) to (C1) of the method of measuring the content ratio of tungsten carbide grains 1 and the content ratio of binder phase 2 in cemented carbide 3. Next, the imaging region is analyzed using the SEM-EDX so as to specify the distribution of the elements specified above in (B1) in the imaging region, thereby obtaining an element mapping image and simultaneously specifying the content ratio of the cobalt in cemented carbide 3. It should be noted that the method of measuring the "content ratio of the cobalt in binder phase 2" is as follows. First, the region in which binder phase 2 is present is specified on the image having been through the binarization processing in the same manner as in (A1) to (F1) of the method of measuring the content ratio of tungsten carbide grains 1 and the content ratio of binder phase 2 in cemented carbide 3. Next, the region in which binder phase 2 is present is analyzed using the SEM-EDX so as to measure the "content ratio of the cobalt in binder phase 2". Further, a method of specifying that "the cobalt in cemented carbide 3 is present only in binder phase 2" is as follows. First, the region in which tungsten carbide grains 1 are present and the region in which binder phase 2 are present are specified on the image having been through the binarization processing in the same manner as in (A1) to (F1) of the method of measuring the content ratio of tungsten carbide grains 1 and the content ratio of binder phase 2 in cemented carbide 3. Next, it is specified that "the cobalt in cemented carbide 3 is present only in binder phase 2", based on the element mapping image and the region in which tungsten carbide grains 1 are present and the region in which binder phase 2 is present.

As long as the applicant has performed the measurement and the measurement is performed onto the same sample, it has been confirmed that measurement results are small in variation and are not intentional even when the cut portion of the cross section of cemented carbide 3 and the imaging region described in (C1) are freely set and the above-described measurement is performed a plurality of times in accordance with the above-described procedure.

Binder phase 2 may further include the first element, and the first element may be at least one element selected from a group consisting of silicon, phosphorus, germanium, tin, rhenium, ruthenium, osmium, iridium, and platinum. Thus, it is possible to provide cemented carbide 3 allowing for a longer tool life of a cutting tool particularly even in cutting of a high-hardness material.

The content ratio of the first element in cemented carbide 3 may be 0.01 mass% or more and 1.0 mass% or less. Thus, binder phase 2 can have both more excellent hardness and more excellent toughness. It should be noted that the content ratio of the first element in binder phase 2 may be 50 mass% or less, 40 mass% or less, 30 mass% or less, 20 mass% or less, 10 mass% or less, or 5 mass% or less. The first element in cemented carbide 3 may be present only in binder phase 2. The lower limit of the content ratio of the first element in cemented carbide 3 may be 0.01 mass% or more, 0.04 mass% or more, or 0.1 mass% or more. The upper limit of the content ratio of the first element in cemented carbide 3 may be 1.0 mass% or less, 0.8 mass% or less, or 0.6 mass% or less. The content ratio of the first element in cemented carbide 3 may be 0.04 mass% or more and 0.8 mass% or less, and may be 0.1 mass% or more and 0.6 mass% or less.

A method of measuring the content ratio of the first element in cemented carbide 3 is as follows. The measurement is performed in the same manner as in the method of measuring the content ratio of the cobalt in cemented carbide 3, except that the "cobalt" is replaced with the "first element". It should be noted that the method of measuring the "content ratio of the first element in binder phase 2" is as follows. The measurement is performed in the same manner as in the method of measuring the "content ratio of the cobalt in binder phase 2", except that the expression "Next, ... so as to measure the "content ratio of the "cobalt" in binder phase 2"" is replaced with the expression "Next, ... so as to measure the "content ratio" of the "first element" in binder phase 2"". Moreover, a method of specifying that "the first element in cemented carbide 3 is present only in binder phase 2" is as follows. The method of specifying that "the cobalt in cemented carbide 3 is present only in binder phase 2" is performed in the same manner except that "Next, ... the "cobalt" in cemented carbide 3 is present only in binder phase 2 is specified" is replaced with "Next, ... it is specified that the "first element" in cemented carbide 3 is present only in binder phase 2".

As long as the applicant has performed the measurement and the measurement is performed onto the same sample, it has been confirmed that measurement results are small in variation and are not intentional even when the cut portion of the cross section of cemented carbide 3 and the imaging region described in (C1) are freely set and the above-described measurement is performed a plurality of times in accordance with the above-described procedure.

In binder phase 2, a percentage {M1/(M1+M2)}×100 of a mass M1 of the first element with respect to a total M1+M2 of mass M1 of the first element and a mass M2 of the cobalt may be 1% or more and 6% or less. Thus, cemented carbide 3 allowing for a longer tool life of a cutting tool particularly even in cutting of a high-hardness material can be provided because binder phase 2 can have both more excellent hardness and more excellent toughness. Here, when the binder phase includes two or more types of the first elements, mass M1 of the first element means the total mass of all the types of the first elements. The lower limit of percentage {M1/(M1+M2)}×100 may be 1% or more, 2% or more, or 3% or more. The upper limit of percentage {M1/(M1+M2)}×100 may be 6% or less, 5% or less, or 4% or less. Percentage {M1/(M1+M2)} ×100 may be 2% or more and 5% or less, and may be 3% or more and 4% or less.

A method of measuring percentage {M1/(M1+M2)}×100 is as follows. The region in which binder phase 2 is present is specified on the image having been through the binarization processing in the same manner as in (A1) to (F1) of the method of measuring the content ratio of tungsten carbide grains 1 and the content ratio of binder phase 2 in cemented carbide 3. The region in which binder phase 2 is present is analyzed using the SEM-EDX, the content ratio of the cobalt and the first element content ratio in binder phase 2 are measured, and percentage{M1/(M1+M2)}×100 is calculated based on these. The above measurement is performed in five different measurement visual fields that do not overlap with one another. In the present specification, the average of percentages "{M1/(M1+M2)}×100" in the five measurement visual fields corresponds to "percentage {M1/(M1+M2)}×100" in binder phase 2.

As long as the applicant has performed the measurement and the measurement is performed on the same sample, it has been confirmed that measurement results are small in variation and are not intentional even when the cut portion of the cross section of cemented carbide 3 and the imaging region described above in (C1) are freely set and the measurement of percentage {M1/(M1+M2)}×100 is performed a plurality of times in accordance with the above-described procedure.

### <Hardness of Binder Phase>

The hardness of binder phase 2 at 25°C as measured by the nanoindenter method is 7.0 GPa or more. Thus, binder phase 2 can have excellent hardness under the condition of 25°C (in other words, under the room temperature condition). The lower limit of the hardness may be 7.1 GPa or more, 7.2 GPa or more, or 7.4 GPa or more. The upper limit of the hardness may be 9 GPa or less, 8.5 GPa or less, or 8 GPa or less. The hardness may be 7.0 GPa or more and 9 GPa or less, 7.1 GPa or more and 8.5 GPa or less, or 7.2 GPa or more and 8 GPa or less.

The hardness of binder phase 2 at 25°C as measured by the nanoindenter method is measured by the nanoindenter method ("Hysitron TI 980 TriboIndenter" provided by Bruker). The nanoindenter method is a method compliant with ISO14577, and is performed under such conditions that a measurement load is 0.5 mN, a loading time is 0.1 second, a load holding time is 0.1 second, and an unloading time is 0.1 second. The measurement target is each of a total of any 10 binder phases 2 exposed by polishing the surface of cemented carbide 3 using a cross session polisher (CP) processing device ("IB-19500CP cross sectional sample production device" (trademark) provided by JEOL). The average value of the respective hardnesses of the total of 10 binder phases 2 is defined as the "hardness of binder phase 2".

As long as the applicant has performed the measurement and the measurement is performed onto the same sample, it has been confirmed that measurement results are small in variation and are not intentional even when 10 binder phases 2 are set freely and the measurement of the hardness of binder phase 2 is performed a plurality of times.

### <<Tungsten Carbide Grains>>

In the first embodiment, tungsten carbide grains 1 include at least either of "pure WC grains (WC containing no impurity element at all and WC in which the content of an impurity element is less than the detection limit are also included)" and "WC grains in each of which an impurity element is intentionally or inevitably contained are included as long as the effects of the present disclosure are not impaired". The content ratio of the impurity in the tungsten carbide grains (when the impurity is constituted of two or more types of elements, the total content ratio of the two or more types of elements) is less than 0.1 mass%. The content ratio of the impurity element in the tungsten carbide grains is measured by the ICP emission spectroscopy (Inductively Coupled Plasma Emission Spectroscopy; measurement device: "ICPS-8100" (trademark) provided by Shimadzu Corporation).

In the first embodiment, the average grain size of tungsten carbide grains 1 is not particularly limited. The average grain size of tungsten carbide grains 1 can be, for example, 0.5 µm or more and 3 µm or less. It has been confirmed that cemented carbide 3 according to the first embodiment can allow for a long tool life regardless of the average grain size of tungsten carbide grains 1.

### <<Application of Cemented Carbide>>

Cemented carbide 3 according to the present embodiment can be used for a cutting tool. Examples of the cutting tool include a cutting tool for general-purpose processing. More specifically, examples of the cutting tool include cutting tools such as a drill, an end mill, an indexable cutting insert for drill, an indexable cutting insert for end mill, an indexable cutting insert for milling, an indexable cutting insert for turning, a metal saw, a gear cutting tool, a reamer, a tap, and the like.

### [Second Embodiment: Method of Producing Cemented Carbide]

The cemented carbide according to the present embodiment can be produced by performing a preparation step for source material powders, a mixing step, a molding step, a sintering step, a cooling step, and a HIP (Hot Isostatic Pressing: hot isostatic pressing method) step in this order. Hereinafter, each step will be described.

### <Preparation Step>

The preparation step is a step of preparing source material powders for the materials to constitute the cemented carbide. Examples of the source material powders include a tungsten carbide powder (hereinafter, also referred to as "WC powder") and a cobalt (Co) powder. In addition to these source material powders, a first element powder, a niobium carbide (NbC) powder, a tungsten carbide (TaC) powder, a titanium carbonitride (TiCN) powder, a zirconium carbide (ZrC) powder, and the like can be prepared. Commercially available powders can be used for these source material powders. The average grain size of these source material powders is not particularly limited, and can be, for example, 0.5 to 2 µm. The average particle size of the source material powders means an average particle size measured by an FSSS (Fisher Sub-Sieve Sizer) method. The average particle size is measured using "Sub-Sieve Sizer Model 95" (trademark) provided by Fisher Scientific.

### <Mixing Step>

The mixing step is a step of mixing, at a predetermined ratio, the source material powders prepared in the preparation step. By the mixing step, a powder mixture in which the source material powders are mixed is obtained. A mixing ratio of the source material powders is appropriately adjusted in accordance with a target composition of the cemented carbide. The first element powder may be used as a source material powder. Thus, the first element is sufficiently dissolved in the binder phase in a solid state, with the result that the cemented carbide is further facilitated to attain a desired "hardness of the binder phase at 25°C as measured by the nanoindenter method". The total content ratio of the WC powder, the Co powder, and the powder other than the first element powder in the powder mixture may be less than 5 mass% from the viewpoint of setting the total of the content ratio of the tungsten carbide grains and the content ratio of the binder phase to fall within a desired range. The content ratio of the binder phase and the content ratio of the WC grains can be set to fall within desired ranges by appropriately adjusting respective amounts of the source material powders to be introduced.

The source material powders can be mixed by using a conventionally known mixing method such as an attritor, a ball mill, or a bead mill. As mixing conditions, conventionally known conditions can be used. A mixing time can be, for example, 2 hours or more and 20 hours or less.

After the mixing step, the powder mixture may be granulated as required. By granulating the powder mixture, the powder mixture is facilitated to be introduced into a die or mold in the molding step described later. For the granulation, a known granulation method can be applied, and a commercially available granulator such as a spray dryer can be used, for example.

### <Molding Step>

The molding step is a step of molding the powder mixture obtained in the mixing step into a shape for a cutting tool so as to obtain a molded body. A molding method and molding conditions in the molding step are not particularly limited and a general method and general conditions are employed.

### <Sintering Step>

The sintering step is a step of sintering the molded body obtained in the molding step so as to obtain a cemented carbide intermediate. Sintering conditions in the present embodiment are as follows. The molded body is heated to 1360°C and is held at 1360°C for 1 hour.

### <Cooling Step>

The cooling step is a step of cooling the cemented carbide intermediate having been through the sintering step. More specifically, the cemented carbide intermediate is cooled to 800°C (hereinafter, also referred to as "first cooling"). A cooling rate of the first cooling is, for example, 20°C/min.

### <HIP Step>

The HIP step is a step of performing a HIP process onto the cemented carbide intermediate having been through the cooling step. Conditions of the HIP step in the present embodiment are as follows. The cemented carbide intermediate is held for 2 hours under a condition of a pressure of 100 MPa. Thus, the cemented carbide according to the first embodiment can be obtained.

### <Features of Method of Producing Cemented Carbide According to the Present Embodiment>

In the present embodiment, the sintering step is performed by heating the molded body to 1360°C and holding the molded body at 1360°C for one hour. Further, the cooling step is performed with the cooling rate until 800°C being set to 20°C/min. Further, the HIP step is performed under conditions of a pressure of 100 MPa and a time of 2 hours. With these steps, the cemented carbide in which the hardness of the binder phase at 25°C as measured by the nanoindenter method is 7.0 GPa or more can be produced. As a result of diligent study, the present inventors have newly found that the cemented carbide according to the present disclosure can be realized by the sintering conditions, the cooling step, and the HIP step.

### [Supplementary Note 1]

In the cemented carbide according to the first embodiment, the nanoindenter method can be performed by a method compliant with ISO14577 under such conditions that a measurement load is 0.5 mN, a loading time is 0.1 second, a load holding time is 0.1 second, and an unloading time is 0.1 second.

### Examples

The present embodiment will be described more specifically with reference to examples. However, the present embodiment is not limited by these examples.

### <<Production of Cemented Carbide>>

Each of cemented carbides according to samples 1 to 19 and 101 to 114 was produced in the following manner.

### <Preparation Step>

As source material powders, a WC powder (average particle size: 1 µm), a Co powder (average particle size: 1 µm), a first element powder, and a TiCN powder (average particle size: 1 µm) were prepared. As the first element powder, a Si powder (average particle size: 1 µm), a Ge powder (average particle size: 1 µm), a Sn powder (average particle size: 1 µm), an Os powder (average particle size: 1 µm), an Ir powder (average particle size: 1 µm), a Pt powder (average particle size: 1 µm), a P powder (average particle size: 1 µm), a Re powder (average particle size: 1 µm), and a Ru powder (average particle size: 1 µm) were prepared.

### <Mixing Step>

The source material powders were mixed at a ratio shown in each of Tables 1 and 2 for 10 hours by using an attritor, thereby obtaining a powder mixture.

### <Molding Step>

The powder mixture was subjected to press molding or extrusion molding, thereby obtaining a molded body having a round bar shape.

### <Sintering Step>

The molded body was heated to a temperature shown in each of Tables 1 and 2, and was held at the temperature for a holding time shown in each of Tables 1 and 2, thereby obtaining a cemented carbide intermediate.

### <Cooling Step>

The cemented carbide intermediate was cooled to 800°C at a cooling rate described in each of Tables 1 and 2.

### <HIP Step>

The cemented carbide intermediate having been through the cooling step was subjected to a HIP process under conditions described in each of Table 1 and Table 2, thereby obtaining the cemented carbide.

Each of the cemented carbides according to samples 1 to 19 and 101 to 114 was produced by the above procedure.

### [Table 1]

**Table 1**

| Sample No. | Mixing Step | | | | | Sintering Step | | Cooling Step | HIP Step | |
|---|---|---|---|---|---|---|---|---|---|---|
| | WC Powder [mass%] | Co Powder [mass%] | First Element Powder [mass%] | Type of First Element | TiCN Powder [mass%] | Temperature [°C] | Holding Time [hour] | Cooling Rate [°C/min] | Pressure [MPa] | Time [hour] |
| 1 | Remainder | 10 | 0.6 | Si | 0 | 1360 | 1 | 20 | 100 | 2 |
| 2 | Remainder | 10 | 0.6 | Ge | 0 | 1360 | 1 | 20 | 100 | 2 |
| 3 | Remainder | 10 | 0.1 | Sn | 0 | 1360 | 1 | 20 | 100 | 2 |
| 4 | Remainder | 10 | 0.6 | Os | 0 | 1360 | 1 | 20 | 100 | 2 |
| 5 | Remainder | 10 | 0.6 | Ir | 0 | 1360 | 1 | 20 | 100 | 2 |
| 6 | Remainder | 10 | 0.6 | Pt | 0 | 1360 | 1 | 20 | 100 | 2 |
| 7 | Remainder | 10 | 0.6 | Si | 4 | 1360 | 1 | 20 | 100 | 2 |
| 8 | Remainder | 10 | 0.5 | Os | 4.3 | 1360 | 1 | 20 | 100 | 2 |
| 9 | Remainder | 1.00 | 0.01 | Si | 0 | 1360 | 1 | 20 | 100 | 2 |
| 10 | Remainder | 10 | 0.5 | P | 0 | 1360 | 1 | 20 | 100 | 9 2 |
| 11 | Remainder | 10 | 0.7 | Si | 0 | 1360 | 1 | 20 | 100 | 2 |
| 12 | Remainder | 10 | 0.1 | Si | 0 | 1360 | 1 | 20 | 100 | 2 |
| 13 | Remainder | 1.00 | 0.01 | P | 0 | 1360 | 1 | 20 | 100 | 2 |
| 14 | Remainder | 10 | 0.09 | Si | 0 | 1360 | 1 | 20 | 100 | 2 |
| 15 | Remainder | 10 | 0.6 | Re | 0 | 1360 | 1 | 20 | 100 | 2 |
| 16 | Remainder | 10 | 0.7 | Si | 0 | 1360 | 1 | 20 | 100 | 2 |
| 17 | Remainder | 12 | 0.6 | Re | 0 | 1360 | 1 | 20 | 100 | 2 |
| 18 | Remainder | 10 | 0.4 | Ru | 0 | 1360 | 1 | 20 | 100 | 2 |
| 19 | Remainder | 10 | 0.65 | Ru | 0 | 1360 | 1 | 20 | 100 | 2 |

### [Table 2]

**Table 2**

| Sample No. | Mixing Step | | | | | Sintering Step | | Cooling Step | HIP Step | |
|---|---|---|---|---|---|---|---|---|---|---|
| | WC Powder [mass%] | Co Powder [mass%] | First Element Powder [mass%] | Type of First Element | TiCN Powder [mass%] | Temperature [°C] | Holding Time [hour] | Cooling Rate [°C/min] | Pressure [MPa] | Time [hour] |
| 101 | Remainder | 1.00 | 0.01 | Os | 0 | 1360 | 1 | 20 | 100 | 2 |
| 102 | Remainder | 10 | 0.6 | P | 0 | 1360 | 1 | 20 | 100 | 2 |
| 103 | Remainder | 10 | 0.6 | Si | 5 | 1360 | 1 | 20 | 100 | 2 |
| 104 | Remainder | 10 | 0 | - | 0 | 1380 | 1 | 10 | 10 | 1 |
| 105 | Remainder | 10 | 0.6 | Re | 0 | 1380 | 1 | 10 | 10 | 1 |
| 106 | Remainder | 10 | 0.6 | Si | 0 | 1380 | 1 | 10 | 10 | 1 |
| 107 | Remainder | 10 | 0.6 | Ge | 0 | 1380 | 1 | 10 | 10 | 1 |
| 108 | Remainder | 10 | 0.6 | Sn | 0 | 1380 | 1 | 10 | 10 | 1 |
| 109 | Remainder | 10 | 0.6 | Os | 0 | 1380 | 1 | 10 | 10 | 1 |
| 110 | Remainder | 10 | 0.6 | Ir | 0 | 1380 | 1 | 10 | 10 | 1 |
| 111 | Remainder | 10 | 0.6 | Pt | 0 | 1380 | 1 | 10 | 10 | 1 |
| 112 | Remainder | 10 | 0.6 | P | 0 | 1380 | 1 | 10 | 10 | 1 |
| 113 | Remainder | 10 | 0.6 | Ru | 0 | 1380 | 1 | 10 | 10 | 1 |
| 114 | Remainder | 0.95 | 0.01 | P | 0 | 1360 | 1 | 20 | 100 | 2 |

### [Table 3]

**Table 3**

| Sample No. | Content Ratio of WC Grains [volume%] | Content Ratio of Binder Phase [volume%] | Total [volume%] | Hardness of Binder Phase [GPa] | Co Content Ratio [mass%] | Content Ratio of First Element [mass%] | {M1/(M1+M2)} ×100[%] | Cutting Test |
|---|---|---|---|---|---|---|---|---|
| | | | | | | | | Cutting Length [m] |
| 1 | Remainder | 19.4 | 100 | 7.5 | 10 | 0.6 | 5.5 | 170 |
| 2 | Remainder | 17.7 | 100 | 7.6 | 10 | 0.6 | 5.5 | 170 |
| 3 | Remainder | 16.4 | 100 | 7.2 | 10 | 0.1 | 1.2 | 160 |
| 4 | Remainder | 16.7 | 100 | 7.6 | 10 | 0.6 | 5.5 | 170 |
| 5 | Remainder | 16.7 | 100 | 7.6 | 10 | 0.6 | 5.6 | 170 |
| 6 | Remainder | 16.7 | 100 | 7.7 | 10 | 0.6 | 5.6 | 170 |
| 7 | Remainder | 16.1 | 89.6 | 8 | 10 | 0.6 | 5.7 | 180 |
| 8 | Remainder | 15.5 | 89 | 7.5 | 10 | 0.5 | 4.9 | 150 |
| 9 | Remainder | 1.8 | 100 | 7.1 | 1.0 | 0.01 | 1 | 150 |
| 10 | Remainder | 19.6 | 100 | 7.4 | 10 | 0.5 | 4.8 | 160 |
| 11 | Remainder | 20.0 | 100 | 7.1 | 10 | 0.7 | 6 | 140 |
| 12 | Remainder | 16.8 | 100 | 7.0 | 10 | 0.1 | 1 | 150 |
| 13 | Remainder | 1.8 | 100 | 7.1 | 1.0 | 0.01 | 1 | 150 |
| 14 | Remainder | 16.7 | 100 | 7.1 | 10 | 009 | 0.9 | 140 |
| 15 | Remainder | 16.7 | 100 | 7.5 | 10 | 0.6 | 58 | 170 |
| 16 | Remainder | 16.7 | 100 | 7.6 | 10 | 0.7 | 6.7 | 140 |
| 17 | Remainder | 16.7 | 100 | 7.4 | 12 | 0.6 | 5.1 | 160 |
| 18 | Remainder | 16.7 | 100 | 7.2 | 10 | 0.4 | 3.7 | 140 |
| 19 | Remainder | 17 | 100 | 7.7 | 10 | 0.65 | 6.1 | 170 |

### [Table 4]

**Table 4**

| Sample No. | Content Ratio of WC Grains [volume%] | Content Ratio of Binder Phase [volume%] | Total [volume%] | Hardness of Binder Phase [GPa] | Content Ratio of Co [mass%] | Content Ratio of First Element [mass%] | {M1/(M1+M2)} ×100[%] | Cutting Test |
|---|---|---|---|---|---|---|---|---|
| | | | | | | | | Cutting Length [m] |
| 101 | Remainder | 1.7 | 100 | 7.2 | 1.0 | 0.01 | 1 | 120 |
| 102 | Remainder | 20.2 | 100 | 7.6 | 10 | 0.6 | 5.7 | 100 |
| 103 | Remainder | 17.8 | 88 | 7.5 | 10 | 0.6 | 5.6 | 110 |
| 104 | Remainder | 16.2 | 100 | 5.8 | 10 | 0 | 0 | 100 |
| 105 | Remainder | 16.6 | 100 | 6.2 | 10 | 0.6 | 5.7 | 110 |
| 106 | Remainder | 16.6 | 100 | 6.8 | 10 | 0.6 | 5.7 | 120 |
| 107 | Remainder | 16.6 | 100 | 6.6 | 10 | 0.6 | 5.7 | 110 |
| 108 | Remainder | 16.6 | 100 | 6.3 | 10 | 0.6 | 5.7 | 100 |
| 109 | Remainder | 16.6 | 100 | 6.7 | 10 | 0.6 | 5.7 | 120 |
| 110 | Remainder | 16.6 | 100 | 6.8 | 10 | 0.6 | 5.7 | 120 |
| 111 | Remainder | 16.6 | 100 | 6.5 | 10 | 0.6 | 5.7 | 110 |
| 112 | Remainder | 20.2 | 100 | 6.2 | 10 | 0.6 | 5.7 | 100 |
| 113 | Remainder | 16.6 | 100 | 6.6 | 10 | 0.6 | 5.7 | 110 |
| 114 | Remainder | 1.8 | 100 | 7.1 | 0.9 | 0.01 | 4.9 | 80 |

### <<Evaluation on Properties of Cemented Carbide>>

### <Content Ratio of Tungsten Carbide Grains>

For the cemented carbide of each sample, the content ratio of the tungsten carbide grains was found by the method described in the first embodiment. Obtained results are shown in the column "Content Ratio of WC Grains [volume%]" in each of Tables 3 and 4. It should be noted that "Remainder" in the column "Content Ratio of WC Grains [volume%]" in each of Tables 3 and 4 means that the content ratio of the tungsten carbide grains is represented by a numerical value equal to a numerical value obtained by subtracting the numerical value described in the column "Content Ratio of Binder Phase [volume%]" in each of Tables 3 and 4 from the numerical value described in the column "Total [volume%]" in each of Tables 3 and 4.

### <Content Ratio of Binder Phase>

For the cemented carbide according to each sample, the content ratio of the binder phase was found by the method described in the first embodiment. Obtained results are shown in the column "Content Ratio of Binder Phase [volume%]" in each of Tables 3 and 4.

### <Hardness of Binder Phase>

For the cemented carbide according to each sample, the hardness of the binder phase was found by the method described in the first embodiment. Obtained results are shown in the column "Hardness of Binder Phase [GPa]" in each of Tables 3 and 4.

### <Content Ratio of Cobalt in Cemented Carbide>

For the cemented carbide according to each sample, the content ratio of the cobalt in the cemented carbide was found by the method described in the first embodiment. Obtained results are shown in the column "Content Ratio of Co [mass%]" in each of Tables 3 and 4. It should be noted that for the cemented carbide according to each sample, it was confirmed by the method described in the first embodiment that the "cobalt in cemented carbide 3 is present only in binder phase 2".

### <Content Ratio of First Element in Cemented Carbide>

For the cemented carbide according to each sample, the content ratio of the first element in the cemented carbide was found by the method described in the first embodiment. Obtained results are shown in the column "Content Ratio of First Element [mass%]" in each of Tables 3 and 4. It should be noted that for the cemented carbide according to each sample, it was confirmed by the method described in the first embodiment that "the first element in cemented carbide 3 is present only in binder phase 2" when the "Content Ratio of First Element [mass%]" was not 0 mass%.
$\left〈\left\{M1/\left(M1+M2\right)\right\}\times 100\right〉$

For the cemented carbide of each sample, {M1/(M1+M2)}×100 was found by the method described in the first embodiment. Obtained results are shown in the column ''{M1/(M1+M2)}×100 [%]" in each of Tables 3 and 4.

### <<Cutting Test>>

First, a round bar consisting of the cemented carbide of each sample was processed to produce, as cutting tools for each sample, three end mills (GSXB20000 type) each having a cutting edge diameter φ of 6 mm. Next, each of the end mills of each sample was used to perform cutting under below-described cutting conditions so as to measure a cutting distance until wear of 0.05 mm is caused in the end mill. For each sample, the average value of cutting distances for the three end mills was calculated to obtain a cutting length. Obtained results are shown in the column "Cutting Length [m]" in each of Tables 3 and 4. It should be noted that it is indicated that as the cutting length is longer, the tool life is longer.

### <Cutting Conditions>

Workpiece: SKD51 (high-hardness material)
Cutting speed Vc: 180 m/min
Feed Fz per cutting edge: 0.15 mm/t
Depth of cut-in Ap: 0.5 mm
Cutting liquid: used (Wet)
The above cutting conditions correspond to cutting of a high-hardness material.

Each of the cemented carbides according to samples 1 to 19 corresponds to an example of the present disclosure. Each of the cemented carbides according to samples 101 to 114 corresponds to a comparative example. In view of the results of Tables 3 and 4, it was found that each of the cemented carbides according to samples 1 to 19 allows for a longer life of a tool even when used as a material of a cutting tool for cutting a high-hardness material, as compared with each of the cemented carbides according to samples 101 to 114.

In view of the above, it was found that each of the cemented carbides according to samples 1 to 19 allows for a longer life of a tool even when used as a material of a cutting tool for cutting a high-hardness material.

Although the embodiments and examples of the present disclosure have been described as described above, it is also initially expected to appropriately combine or variously modify the configurations of the above-described embodiments and examples.

The embodiments and examples disclosed herein are illustrative and non-restrictive in any respect. The scope of the present invention is defined by the terms of the claims, rather than the embodiments and examples described above, and is intended to include any modifications within the scope and meaning equivalent to the terms of the claims.

### REFERENCE SIGNS LIST

1 tungsten carbide grain; 2 binder phase; 3 cemented carbide

## Claims

1. A cemented carbide comprising a plurality of tungsten carbide grains and a binder phase, wherein
the cemented carbide includes 89 volume% or more of the tungsten carbide grains and the binder phase in total,
the cemented carbide includes 1.8 volume% or more and 20.0 volume% or less of the binder phase,
the binder phase includes cobalt,
the cemented carbide includes 1.0 mass% or more of the cobalt, and
a hardness of the binder phase at 25°C as measured by a nanoindenter method is 7.0 GPa or more.

2. The cemented carbide according to claim 1, wherein
the binder phase further includes a first element, and
the first element is at least one element selected from a group consisting of silicon, phosphorus, germanium, tin, rhenium, ruthenium, osmium, iridium, and platinum.

3. The cemented carbide according to claim 2, wherein in the binder phase, a percentage {M1/(M1+M2)}×100 of a mass M1 of the first element with respect to a total M1+M2 of the mass M1 of the first element and a mass M2 of the cobalt is 1% or more and 6% or less.
